

# United States Patent [19]

Blytas

[11] Patent Number: 4,705,531

[45] Date of Patent: Nov. 10, 1987

[54] REDUCTION OF SODIUM IN COAL BY  
WATER WASH FOLLOWED BY ION  
EXCHANGE WITHIN A PIPELINE

[75] Inventor: George C. Blytas, Houston, Tex.

[73] Assignee: Shell Oil Company, Houston, Tex.

[21] Appl. No.: 779,717

[22] Filed: Sep. 24, 1985

[51] Int. Cl.<sup>4</sup> ..... C10L 9/02

[52] U.S. Cl. ..... 44/1 R; 423/461

[58] Field of Search ..... 44/1 R, 5 R; 201/17;  
423/461

## [56] References Cited

### U.S. PATENT DOCUMENTS

3,993,456 11/1976 Cole et al. ..... 44/1 SR  
3,998,604 12/1976 Hinkley ..... 44/1 R

4,053,285 10/1977 Robinson et al. ..... 44/1 SR  
4,076,607 2/1978 Zavitsanos et al. ..... 44/1 SR  
4,204,843 5/1980 Neavel ..... 44/1 R

Primary Examiner—Carl F. Dees

Attorney, Agent, or Firm—H. W. Coryell; D. Y. Wolfs

## [57] ABSTRACT

A coal or similar carbonaceous fuel is selectively freed of sodium by water washing it and ion exchanging the washed coal with a strong aqueous electrolyte solution which is substantially free of sodium ions and contains a kind and concentration of ions which are correlated with the composition of the coal to cause a selective removal of ion-exchangeable sodium from the coal, with at least a significant proportion of the ion-exchanging being conducted within a pipeline.

10 Claims, No Drawings

**REDUCTION OF SODIUM IN COAL BY WATER WASH FOLLOWED BY ION EXCHANGE WITHIN A PIPELINE**

**RELATED APPLICATIONS**

The present application is related to my commonly assigned and concurrently filed applications, Ser. Nos. 779,716 and 779,718 (now abandoned) on "Reduction of Sodium in Coal by Water Wash and Ion Exchange with Weak Electrolyte" and "Selective Reduction of Sodium in Coal by Water Wash and Ion Exchange with Tailored Electrolyte".

**BACKGROUND OF THE INVENTION**

The present invention relates to upgrading coal by removing sodium ions. More particularly, the invention relates to removing sodium ions from coal by means of water-washing and ion-exchanging.

The presence of large amounts of sodium in coal is undesirable as it contributes to fouling of combustion facilities. The fouling problems can arise if sodium exceeds about 3%w (as  $\text{Na}_2\text{O}$ ), yet several important deposits of coal contain considerably more than that much sodium. Thus, a process which can economically remove, for example, 30-70% of the sodium, can be very desirable and can be a prerequisite condition for exploitation of sizeable deposits.

The levels of sodium oxide in the ash at which coal combustion can lead to fouling problems are not yet clearly defined, and can be different for different coals. Nevertheless, levels in excess of about 3%w are not desirable and coals with more than 4%w in the ash, are generally difficult to market. Some Powder River Basin coal samples have been found to yield over 6%w of sodium oxide. And, coals with sodium oxide contents in excess of 8 or 9%w have also been found and documented.

U.S. Department of Energy publication DOE/G-FETY/RI-82/3 "Conceptual Design of a 1.6 MM Tons/Year Lignite Preparation Facility for Sodium Reduction" describes ion exchanges of coal with 0.11 normal sulfuric acid for various times and solid to liquid ratios and indicates that a sodium oxide content decreased from 8.5 to 0.99% and the selectivity of the ion removal varied with variations in residence time.

A publication from Pennsylvania State University Fuel Science Program "Ion Exchange in Selected Low Rank Coals, Part I Equilibrium, Part II Kinetics", Solvent Extraction, Ion Exchange, 1:4, 813-825 (1983), describes measurements of equilibrium ion exchange behavior for metal cations with hydrogen ions and indicates the exchange to be a linear function of pH regardless of the cation concentration of the solution; with the extent of exchange being a function of available hydrogen ions.

**SUMMARY OF THE INVENTION**

The present invention relates to an improved ion exchange process for reducing the sodium content of coal. The coal is first washed with water that is substantially free of sodium ions, for removing water-soluble materials containing sodium ions. The washed coal is then ion exchanged with an aqueous solution of strong electrolyte solution in which both kinds and concentrations of ions are correlated with the kind and concentration of ion exchangeable cations on the coal. The electrolyte solution used in the ion exchange (a) is relatively

free of sodium ions, (b) is sufficiently free of substances capable of forming atmospheric pollutants during the oxidation of coal so that the resultant total amount of those substances in the ion exchange coal is insufficient to cause significant pollution, and (c) contains cations capable of exchanging with ion exchangeable cations on the coal in an amount which is less than the stoichiometric amount of the cations on the coal but is an amount which causes sodium ions to be removed selectively from the coal.

In a preferred procedure, at least a significant proportion of the ion exchange treatment is effected by flowing within a pipeline both a solution of a slurry of coal and aqueous fluid which is substantially free of sodium ions, and a stream of a fluid which contains sufficient compounds capable of forming an aqueous solution of a strong or weak electrolyte to provide an electrolyte solution having the properties designated (a), (b) and (c) when mixed with the aqueous phase of the coal slurry.

An initial portion of the ion exchange treatment can advantageously be conducted by contacting the water washed coal with an aqueous solution of strong electrolyte in a first location before conducting additional ion exchange treatment within a pipeline. In such a procedure, it is further advantageous to use, as at least one of the compounds capable of forming an aqueous electrolyte a compound which is capable of forming a weak acid electrolyte.

The advantages of the present invention are many fold. Some of these advantages are: (a) the consumption of exchanging reagent can be kept at an economically acceptable low level; (b) the process is selective in removing sodium rather than calcium and magnesium, which are often useful as sulfur oxide capturing species; (c) the spent solutions do not leave a very low pH, and thus are relatively non-corrosive and easy to dispose of; and (d) the process can be adapted or tailored to suit a wide variety of coals, by determining their cationic concentration and adjusting the composition and concentration of the ion exchanging solution as described herein.

**DESCRIPTION OF THE INVENTION**

We have found that sodium may occur in coals in three forms; (a) water-soluble sodium, (b) ion-exchangeable sodium, and (c) fixed sodium. The ion-exchangeable sodium can be about 30 to 80 percent of the total, with the balance split between water-soluble and fixed sodium. Many low-rank coals can be rendered marketable and usable by the present process, which is often capable of removing 30 to 70 percent of the sodium ions (measured as  $\text{Na}_2\text{O}$ ) economically. This invention is illustrated by using a coal sample from the Powder River Basin. However, the invention is not limited to coals of this origin, and the method disclosed herein is readily adaptable to essentially any coal or lignite characterized by a high sodium level.

A sample of coal from the Powder River Basin was ground into three fractions as follows:

- (A)  $\frac{3}{4}$ " by 28 mesh
- (B) Less than 14 mesh
- (C) Less than 28 mesh

Sample fractions (B) and (C) were dried to 8-9%w water (down from ~25%) by heating in a vacuum at 100° C. Analysis of sample fractions (B) and (C) has yielded  $\text{Na}^+$   $\text{Mg}^{++}$  and  $\text{Ca}^{++}$  contents and ash levels which were less than 3% apart. Accordingly, for the

metal removal calculations, we have used the average of analyses obtained on sample fractions (B) and (C).

We can consider the coal sample as an ion-exchanger in which negative fixed sites (believed to be R—COO<sup>-</sup> or similar moieties) are counterbalanced by ion-exchangeable cations, primarily by Na<sup>+</sup>, Ca<sup>++</sup> and Mg<sup>++</sup> ions. Relatively minor amounts of K<sup>+</sup> ion and other metal ions are also present, but will be neglected in the present context. The form in which iron occurs has not been determined, although it is expected to be primarily as pyrite. In Table 1, along with the analysis of Na<sup>+</sup>, Ca<sup>++</sup> and Mg<sup>++</sup>, we show the percentage of base capacity contributed by each of these cations.

TABLE 1

|                 | Metal and Ash Contents of the Coal Tested |          |         | Equivalent Base Capacity % |
|-----------------|-------------------------------------------|----------|---------|----------------------------|
|                 | 14-28 Mesh                                | <28 Mesh | Average |                            |
| Sodium (ppm)    | 2370                                      | 2430     | 2400    | 17                         |
| Calcium (ppm)   | 7570                                      | 7800     | 7685    | 64                         |
| Magnesium (ppm) | 1330                                      | 13700    | 1350    | 19                         |
| Ash % w         | 4.79                                      | 4.77     | 4.78    | —                          |

Contact times from a few hours to several days were studied, the former corresponding to mine-mouth conditions, the latter corresponding to pipeline transport conditions. Coal particle sizes and solid/liquid ratios were selected accordingly.

The degree of sodium, calcium and magnesium reduction in coal, resulting from various ion-exchange treatments, was estimated by monitoring the increase in the level of these ions in the treating solution. In general, Na<sup>+</sup> analysis was done by ion-specific electrode methods, whereas Ca<sup>++</sup> and Mg<sup>++</sup> analysis was done by titration methods.

Sodium reduction by exchange with strong electrolytes was studied using sulfuric acid, H<sub>2</sub>SO<sub>4</sub>, and calcium chloride, CaCl<sub>2</sub>. Three levels of stoichiometry were investigated, in three sets of experiments, as follows:

Set 1 Using 200% of the stoichiometric amount of ion-exchangeable cations on the coal, i.e., using twice as many equivalents of H<sup>+</sup>, or Ca<sup>++</sup> as the total Na<sup>+</sup>+Ca<sup>++</sup>+Mg<sup>++</sup> equivalents in the coal.

Set 2 Using 68% of the stoichiometric amount, which is less than the total equivalent present in the coal but more than the most abundant cation, calcium, which accounts for 64% of the coal capacity, and

Set 3 Using, 23% of the stoichiometric amount, which is still 35% more than the equivalent of sodium present in the coal.

The removal of Na<sup>+</sup> or other ions achieved in these three Sets was compared with the extent of removal achieved by water washing. This latter figure yields the amount of sodium associated with water-soluble salts adhering to the coal as crystalline salts or dissolved salts.

Tables 2 and 3 summarize the results obtained in experimental Set-1, at 200% of stoichiometric addition of the exchange agent. The Tables also show the effect of washing with water only. It should be noted that the equilibrium pH with the H<sub>2</sub>SO<sub>4</sub> experiments (i.e., ion-exchanges with an aqueous solution containing a 100% excess of cations capable of exchanging with ion-exchangeable cations on the coal) was less than 1, whereas the water and CaCl<sub>2</sub> treatments yielded solutions of nearly neutral pH. All of these tests were car-

ried out using 3/1 liquid/solid ratios. The large excess of reagents in these tests make them useful as "reference tests," but too high for consideration in a practical sodium reduction process.

Table 2 shows that 78 to 81% of the Na<sup>+</sup> is removed with excess H<sub>2</sub>SO<sub>4</sub> reagent in two days. Since water wash alone brings about 20±1% reduction, we can conclude that the maximum exchangeable Na<sup>+</sup> ion is Ca. 60% of the total. From the data in Table 2, we also conclude that about 19% of the sodium is associated with species which are insoluble even in excess 0.2N H<sub>2</sub>SO<sub>4</sub> solution.

In experimental Set-1 (200% stoichiometric) CaCl<sub>2</sub> was marginally less efficient than H<sub>2</sub>SO<sub>4</sub> in sodium reduction. It is not clear whether this is a real difference in reagent effectiveness, or a reflection of the difficulty associated with Na<sup>+</sup> determinations in the presence of a large excess of Ca<sup>++</sup> ions.

In Set-1 experiments, water wash yielded essentially no Ca<sup>++</sup> or Mg<sup>++</sup> ion leaching. Thus, those species either are not present as water soluble salts in the aqueous phase adhering on the ground-up, partially dried coal samples or, if they are present as soluble salts, there is a high affinity for adsorption of such salts on the coal.

Table 3 shows the extraction of Ca<sup>++</sup> ions by H<sub>2</sub>SO<sub>4</sub>. An interesting observation is noted for samples B and C in this Table, i.e., with the samples which had been ground-up. In these samples, the calcium ion concentration goes through a maximum in 1 to 2 hours. This trend must be due to changes in solubility and adsorptivity of CaSO<sub>4</sub> species. Apparently, the solubility of CaSO<sub>4</sub> decreases with decreasing acidity of the solution, i.e., decreases as the exchange of base metal by H<sup>+</sup> proceeds to completion after the first 2 or so hours. The coarser sample did not show this effect.

TABLE 2

| Contact Time<br>(hours) | Sodium Reduction (%) by Treatment with 100% Excess H <sub>2</sub> SO <sub>4</sub> and CaCl <sub>2</sub> and With Water |    |     |                 |    |     |                 |    |     |
|-------------------------|------------------------------------------------------------------------------------------------------------------------|----|-----|-----------------|----|-----|-----------------|----|-----|
|                         | (A)<br>1/2" by 28 Mesh                                                                                                 |    |     | (B)<br>-14 Mesh |    |     | (C)<br>-28 Mesh |    |     |
|                         | I                                                                                                                      | II | III | I               | II | III | I               | II | III |
| 0.8                     | 48                                                                                                                     | 25 | 16  | 73              | 60 | 16  | 78              | 59 | 18  |
| 2.4                     | 53                                                                                                                     | 33 | 18  | 75              | 60 | 17  | 80              | 60 | 18  |
| 24                      | 61                                                                                                                     | 65 | 19  | —               | —  | 19  | 81              | —  | 19  |
| 48                      | 77                                                                                                                     | 66 | 21  | 78              | 66 | 21  | 81              | 66 | 22  |

Conditions

Liquid to Solid Ratio: 3 to 1

Solutions:

I = 0.4 N H<sub>2</sub>SO<sub>4</sub>

II = 0.4 N CaCl<sub>2</sub>

III = Deionized water

Na<sup>+</sup> analysis in ppmw

Ambient temperature with shaking

TABLE 3

| Contact time (hrs) | Calcium Reduction (%) by Treatment With 100% Excess of H <sub>2</sub> SO <sub>4</sub> |                 |                 |
|--------------------|---------------------------------------------------------------------------------------|-----------------|-----------------|
|                    | Sample                                                                                |                 |                 |
|                    | (A)<br>1/2" by 28 Mesh                                                                | (B)<br>-14 Mesh | (C)<br>-28 Mesh |
| 0.2                | 3                                                                                     | 38              | 37              |
| 0.8                | 17                                                                                    | 50              | 50              |
| 2.4                | 18                                                                                    | 46              | 40              |
| 24                 | 22                                                                                    | 24              | 23              |

TABLE 3-continued

| Calcium Reduction (%) by Treatment With 100% Excess of $H_2SO_4$ |                        |                 |                 |
|------------------------------------------------------------------|------------------------|-----------------|-----------------|
| Contact time (hrs)                                               | Sample                 |                 |                 |
|                                                                  | (A)<br>1/2" by 28 Mesh | (B)<br>-14 Mesh | (C)<br>-28 Mesh |
| 48                                                               | 23                     | 24              | 23              |

Conditions:  
Liquid to Solid Ratio: 3 to 1  
Solution: 0.4 N  $H_2SO_4$   
Shaking at 23° C.

In experimental Set-2 (with 68% of the stoichiometric amount of reagent), the amount of cations is still 4-times the amount needed to exchange all of the  $Na^+$  ion present at high selectivity. In this set, only -14 mesh coal was used, and long contact times were studied to simulate pipeline transport conditions more closely.

The results from experimental Set-2 are shown in Tables 4 and 5. The  $Na^+$  reductions achieved with this dosage compares favorably with those achieved with the four times higher reagent dosages in Set-1 (200%). From a process standpoint, an additional advantage over Set-1 is that the pH levels at equilibration are higher in Set-2 than in Set-1. Thus, the final pH region with  $H_2SO_4$  exchanges shown in Table 2 is ca. 0.8 after 48 hours, whereas the pH obtained with  $H_2SO_4$  exchange in Table 4, is 2.9 after 10 minutes, 4.1 after 45 minutes, and 5.3 after 2.4 hours. This last high pH value also suggests that the normality of the treating solution was reduced from 0.1N initially to ca. 0.00001N, thus indicating that essentially all of the  $H^+$  ion available was consumed to exchange cations from coal.

With regard to sodium reduction, Set-2 results agree closely with those of Set-1 (compare to Tables 2 and 4). A notable difference is that 0.1N  $CaCl_2$  appears to be a more effective exchanger than 0.4N  $CaCl_2$ . It is, however, also possible that the  $Na^+$  analysis in Set-2 is more accurate, because the  $Ca^{++}$  level at the end of exchange was very low (unlike in Set-1).

With regard to the exchange of  $Ca^{++}$  and  $Mg^{++}$ , Table 5 shows again a maximum of exchange in the first 2 to 3 hours, with a subsequent gradual reduction over the next 2 to 3 days. This trend has been observed with other samples as well and appears to be a characteristic of  $Ca^{++}$  and  $Mg^{++}$  exchange by  $H_2SO_4$ . This type of behavior should be considered when selecting conditions for an optimal ion exchange of coal.

Table 6 shows further how the level of  $Na^+$  ion in solution increases with time, whereas the levels of  $Ca^{++}$  and  $Mg^{++}$  in solution decrease with time. The percentage of  $Na^+ + Mg^{++} + Ca^{++}$  which migrate from the coal into the solution decrease from 59% of the total coal base in 0.8 hours to 40% in 92 hours. In Table 6, the sodium present in solution is 82% of the total, about the same as reflected in Table 4.

TABLE 4

| Contact Time (Hrs) | Na <sup>+</sup> Exchange with 68% of Stoichiometric $H_2SO_4$ and $CaCl_2$ Solutions and Water |                                                          |        |
|--------------------|------------------------------------------------------------------------------------------------|----------------------------------------------------------|--------|
|                    | 0.1 N $H_2SO_4$<br>Percent $Na^+$ Exchanged and/or Washed                                      | 0.1 N $CaCl_2$<br>Percent $Na^+$ Exchanged and/or Washed | $H_2O$ |
| 0.2                | 63                                                                                             | 51                                                       | 18     |
| 0.8                | 76                                                                                             | 76                                                       | 19     |
| 2.4                | 76                                                                                             | 77                                                       | 18     |
| 24                 | 80                                                                                             | 80                                                       | 20     |

TABLE 4-continued

| Contact Time (Hrs) | Na <sup>+</sup> Exchange with 68% of Stoichiometric $H_2SO_4$ and $CaCl_2$ Solutions and Water |                                                          |        |
|--------------------|------------------------------------------------------------------------------------------------|----------------------------------------------------------|--------|
|                    | 0.1 N $H_2SO_4$<br>Percent $Na^+$ Exchanged and/or Washed                                      | 0.1 N $CaCl_2$<br>Percent $Na^+$ Exchanged and/or Washed | $H_2O$ |
| 48                 | 80                                                                                             | 80                                                       | 22     |
| 92                 | 81                                                                                             | 81                                                       | 23     |

Liquid to Solid Ratio: 3 to 1  
Particle Size less than 14 mesh

TABLE 5

| Ca <sup>++</sup> and Mg <sup>++</sup> Exchange Using 68% of Stoichiometric $H_2SO_4$ Solution |                             |                             |
|-----------------------------------------------------------------------------------------------|-----------------------------|-----------------------------|
| Contact Time (Hours)                                                                          | Ca <sup>++</sup> Exchange % | Mg <sup>++</sup> Exchange % |
| 0.2                                                                                           | 36                          | 94                          |
| 0.8                                                                                           | 46                          | 96                          |
| 2.4                                                                                           | 47                          | ~100                        |
| 24                                                                                            | 26                          | 91                          |
| 48                                                                                            | 25                          | 83                          |
| 92                                                                                            | 24                          | 57                          |

Liquid to Solid Ratio: 3 to 1  
0.1 N  $H_2SO_4$  Solution  
Particle Size <14 Mesh.

TABLE 6

| Time (Hours) | Percentage of Coal Base Found in Solution after 0.8 and 92 hours |         |           |
|--------------|------------------------------------------------------------------|---------|-----------|
|              | Sodium                                                           | Calcium | Magnesium |
| 0.8          | 13                                                               | 29      | 17        |
| 92           | 14                                                               | 15      | 11        |
| Maximum      | 17                                                               | 64      | 19        |
|              |                                                                  |         | Total     |
|              |                                                                  |         | 59        |
|              |                                                                  |         | 40        |
|              |                                                                  |         | 100       |

The results obtained in Experimental Set-3 (with 23% of the stoichiometric amounts) are summarized in Tables 7 and 8. These experiments were performed at a 3 to 1 liquid to solid ratio with 0.03N  $H_2SO_4$  or  $CaCl_2$ . These dosages correspond to a 35% excess over the sodium level present.

TABLE 7

| Contact Time (hours) | Na <sup>+</sup> and Ca <sup>+</sup> Exchange with $H_2SO_4$ at 23% of Stoichiometric Ratio |                            |
|----------------------|--------------------------------------------------------------------------------------------|----------------------------|
|                      | Na <sup>+</sup> Exchange %                                                                 | Ca <sup>+</sup> Exchange % |
| 0.2                  | 56                                                                                         | 12                         |
| 0.8                  | 60                                                                                         | 12                         |
| 2.4                  | 62                                                                                         | 11                         |
| 24                   | 65                                                                                         | 11                         |
| 48                   | 68                                                                                         | 11                         |

Liquid to Solid Ratio: 3 to 1  
0.03 N  $H_2SO_4$  Solution

TABLE 8

| Contact Time (hours) | Displacement of $Na^+$ by 23% of Stoichiometric $CaCl_2$ Solution |  |
|----------------------|-------------------------------------------------------------------|--|
|                      | Percent Exchanged                                                 |  |
| 0.2                  | 54                                                                |  |
| 0.8                  | 59                                                                |  |
| 2.4                  | 60                                                                |  |
| 48                   | 65                                                                |  |

Liquid to Solid Ratio: 3 to 1

Tables 7 and 8 show that  $Na^+$  is displaced more completely than  $Ca^{++}$  by  $H_2SO_4$ . However, both,  $H_2SO_4$  and  $CaCl_2$  can displace over 60% of the  $Na^+$  in 2.4 hours (Table 8).

In Table 7, the displacement of  $Na^+$  corresponds to 12% of the total available base, whereas that of  $Ca^{++}$  corresponds to 8%. We can define a selectivity for

Na<sup>+</sup> versus Ca<sup>++</sup> + Mg<sup>++</sup> removal by comparing the relative amounts of Na<sup>+</sup> removed to those of Ca<sup>++</sup> + Mg<sup>++</sup>. Such a definition would suggest that the lower concentrations of H<sub>2</sub>SO<sub>4</sub> are more effectively utilized in Na-reduction than the higher concentrations of H<sub>2</sub>SO<sub>4</sub>.

Quantitatively, we can define the selectivity ( $\beta$ ) for Na<sup>+</sup> over Ca<sup>++</sup> + Mg<sup>++</sup> as follows:

$$\beta = \frac{\text{% of total base capacity (TBC) extracted as Na}^+}{\text{% of TBC accounted by Na}^+ \text{ in coal}} = \frac{\text{% of TBC extracted as Ca}^{++} + \text{Mg}^{++}}{\text{% of TBC accounted by Ca}^{++} + \text{Mg}^{++} \text{ in coal}}$$

In Table 9, this ratio,  $\beta$ , is given for the three sets of experiments, using the longest contact time results in each one. The selectivity goes from 1.94 at 200% stoichiometric, through 2.54 at 68% stoichiometric, to 8 at 23% stoichiometric. The corresponding reductions of sodium achieved are 80%, 80% and 68%. These results show clearly that we can achieve a significant degree of sodium reduction, using only moderate amounts of ion exchange reagent. The concept of selective use of a reagent for sodium reduction can be used to arrive at near optimal process conditions, either for mine-mouth or for coal slurry pipeline application.

TABLE 9

| Selectivity of H <sub>2</sub> SO <sub>4</sub> for Na <sup>+</sup> versus Ca <sup>++</sup> + Mg <sup>++</sup> Removal |         |                             |
|----------------------------------------------------------------------------------------------------------------------|---------|-----------------------------|
| H <sub>2</sub> SO <sub>4</sub> Excess over Stoichiometric <sup>(a)</sup>                                             | $\beta$ | % Na <sup>+</sup> Reduction |
| 200%                                                                                                                 | 1.94    | 80                          |
| 68%                                                                                                                  | 2.54    | 80                          |
| 23%                                                                                                                  | 8.0     | 68                          |

<sup>(a)</sup>Estimated on the basis of Total Base Capacity (TBC) of Na<sup>+</sup> + Ca<sup>++</sup> + Mg<sup>++</sup>

In order to assess the effect of background Na<sup>+</sup> ions on the washing and ion exchange capacity of water and H<sub>2</sub>SO<sub>4</sub> solutions we have added background concentrations of 0.04% w Na<sub>2</sub>SO<sub>4</sub> (130 ppm Na<sup>+</sup>) and 0.1% w Na<sub>2</sub>SO<sub>4</sub> (320 ppm Na<sup>+</sup>) in deionized water or in 0.01N H<sub>2</sub>SO<sub>4</sub> reagents and studied Na<sup>+</sup> reduction in 1 and 2 hours. The results shown in Table 10, show that at low reagent concentrations (justified by the high liquid/solid ratios), the Na<sup>+</sup> would have an adverse effect on Na<sup>+</sup> reduction in a mine-mouth operation (short contact times, high liquid/solid ratios).

The results shown in Table 10 were obtained at a relatively high Na<sup>+</sup> level (130 and 320 ppm) and with low H<sub>2</sub>SO<sub>4</sub> normality. A second experiment was carried out in which both Na<sup>+</sup> and Ca<sup>++</sup> were added as background cations at 100 ppm each and the concentration of H<sub>2</sub>SO<sub>4</sub> was raised to 0.025N and to 0.05N. A liquid to solid ratio of 6 was used. The results, summarized in Table 11, show that sodium reduction in this case is in the range of 60 to 70% in three hours, i.e., acceptable for most process applications.

TABLE 10

| Aqueous Phase                                                                                                               | Effect of Na <sup>+</sup> Level in Solution on Na <sup>+</sup> Reduction |       |
|-----------------------------------------------------------------------------------------------------------------------------|--------------------------------------------------------------------------|-------|
|                                                                                                                             | 1 HR                                                                     | 2 HRS |
| Deionized Water                                                                                                             | 23                                                                       | 25    |
| Deionized Water + 0.04% w Na <sub>2</sub> SO <sub>4</sub>                                                                   | 19                                                                       | 23    |
| Deionized Water + 0.1% w Na <sub>2</sub> SO <sub>4</sub>                                                                    | <10                                                                      | 12    |
| 0.01 N H <sub>2</sub> SO <sub>4</sub>                                                                                       | 50                                                                       | 59    |
| 0.01 N H <sub>2</sub> SO <sub>4</sub> + 0.04% w Na <sub>2</sub> SO <sub>4</sub> (0.0056 N Na <sub>2</sub> SO <sub>4</sub> ) | 39                                                                       | 56    |
| 0.01 N H <sub>2</sub> SO <sub>4</sub> +                                                                                     | 20                                                                       | 32    |

TABLE 10-continued

| Aqueous Phase                                                                     | Effect of Na <sup>+</sup> Level in Solution on Na <sup>+</sup> Reduction |                                    |
|-----------------------------------------------------------------------------------|--------------------------------------------------------------------------|------------------------------------|
|                                                                                   | % Na <sup>+</sup> Removal<br>1 HR                                        | % Na <sup>+</sup> Removal<br>2 HRS |
| 0.1% w Na <sub>2</sub> SO <sub>4</sub> (0.014 N Na <sub>2</sub> SO <sub>4</sub> ) |                                                                          |                                    |

Liquid to solid ratio: 6 to 1

All values are  $\pm 14\%$  of the reported removal, due to analytical difficulties resulting from the use of high levels of Na<sup>+</sup> background in the sample.

TABLE II

| Contact Time<br>(Hrs) | Sodium Reduction Using H <sub>2</sub> SO <sub>4</sub> in the Presence of Sodium and Calcium Ions Background cations in reagent solutions:<br>100 ppm Na <sup>+</sup> , 100 ppm Ca <sup>++</sup> |        |    |    |
|-----------------------|-------------------------------------------------------------------------------------------------------------------------------------------------------------------------------------------------|--------|----|----|
|                       | Solution                                                                                                                                                                                        |        |    |    |
|                       | 0.025 N                                                                                                                                                                                         | 0.05 N |    |    |
| 1                     | 49                                                                                                                                                                                              | 16     | 60 | 31 |
| 2                     | 59                                                                                                                                                                                              | 14     | 66 | 35 |
| 3                     | 61                                                                                                                                                                                              | 14     | 71 | 37 |

Liquid to solid ratio: 6 to 1

Reduction results are  $\pm 8\%$  of the reported value.

Comparison of the results in Tables 10 and 11 suggests that the ionic composition of the water used to make the exchange solutions should be considered in some process applications. However, at higher ratios (H<sup>+</sup> + Ca<sup>++</sup>)/(Na<sup>+</sup>) the effect of background sodium on sodium displacement becomes less critical.

The present process is preferably conducted in two steps, for example, 1 hour low pressure, open vessel mine-mouth contact at a 6 to 1 liquid to solid ratio, followed by a pipeline transport step at a 1.5 to 1 liquid to solid ratio, optionally at high pressure.

In simulating this process a portion of the -14 mesh size coal was screened to yield a fraction of size large enough so that a coal/water separation can be easily brought about after the first "mine-mouth" contacting step. This entails separating the -14 mesh coal using a 100 mesh screen. It yields a large particles fraction ranging from 150 microns to 1400 microns in size, and a small particles fraction with less than 100 micron size. The size classification in the -14 mesh sample yielded 74.2% w larger than 100 mesh and 25.8% w smaller than 100 mesh.

The larger fraction was treated in the 1-hour treatment steps and the solids were separated from the liquid. The entire sample was then treated for 4 days. A 14-day contact time would yield higher Na<sup>+</sup> exchange. However, for comparative purposes the shorter contact time was selected as possibly being more informative, in that rates would tend to play a more important role than in a longer experiment.

The reagents for the open vessel, 1-hour treatment, were the following:

- (A) Deionized water
- (B) Deionized water/dry ice (providing a weak electrolyte)
- (C) 0.01N H<sub>2</sub>SO<sub>4</sub> in deionized water
- (D) 0.01N acetic acid in deionized water (providing a weak electrolyte)

In all of these tests a 6 to 1 liquids to solids ratio was used. After 1 hour of contact the solids and liquids were separated and the "pipeline transport" experiment was done using either deionized water, or water/high pressure CO<sub>2</sub>. In one case, (C), a 0.01N H<sub>2</sub>SO<sub>4</sub> treatment

was also tested. Thus, a total of nine experiments simulating pipeline conditions were carried out. In all of these, a 1.5 to 1 liquid to solid ratio was used. The results of these experiments are summarized in Table 12.

TABLE 12

| Treatment                                           | Cumulative % Removal of Na <sup>+</sup> Calculated on the Basis of Total Coal Sample |         |         |
|-----------------------------------------------------|--------------------------------------------------------------------------------------|---------|---------|
|                                                     | Step I                                                                               | Step II | Run No. |
| (A) Deionized Water                                 | 10.2                                                                                 |         |         |
| (a) Deionized water                                 |                                                                                      | 16.5    | 1       |
| (b) Deionized water + High Pressure CO <sub>2</sub> |                                                                                      | 36      | 2       |
| (B) Deionized Water + Dry Ice                       | 26                                                                                   |         |         |
| (a) Deionized water                                 |                                                                                      | 28      | 3       |
| (b) Deionized water + High Pressure CO <sub>2</sub> |                                                                                      | 40      | 4       |
| (C) 0.01 N H <sub>2</sub> SO <sub>4</sub>           | 31.4                                                                                 |         |         |
| (a) Deionized water                                 |                                                                                      | 32      | 5       |
| (b) Deionized water + High Pressure CO <sub>2</sub> |                                                                                      | 43      | 6       |
| (c) 0.01 N H <sub>2</sub> SO <sub>4</sub>           |                                                                                      | 38      | 7       |
| (D) 0.01 N Acetic Acid                              | 28.2                                                                                 |         |         |
| (a) Deionized water                                 |                                                                                      | 30      | 8       |
| (b) Deionized water + High Pressure CO <sub>2</sub> |                                                                                      | 40      | 9       |

Review of the results in Table 12 shows that a deionized water only case (A)(a), would yield a marginal removal of Na<sup>+</sup> of about 16-17% (Run No. 1). On the other hand, using 0.01N H<sub>2</sub>SO<sub>4</sub> in the first step and high CO<sub>2</sub> pressure in the second step yields 43% Na<sup>+</sup> removal (Run No. 6).

No extractions with CaCl<sub>2</sub> have been carried in the process context discussed here. However, CaCl<sub>2</sub>, if used at levels that would not increase the chlorine levels in coal above those acceptable, would be a promising cation exchange material. The maximum dosage of CaCl<sub>2</sub> tolerable would be higher when the coal treated is low on chlorine to begin with.

In general the present invention can advantageously be applied to substantially any type of coal and/or lignite, or other solid carbonaceous fuel having an undesirably high sodium content such as 4% or more sodium oxide in the ash. Such materials are referred to herein by the term "coal".

The aqueous solution of strong electrolytes with which the coal is ion exchanged can be compounded in substantially any manner as long as the resulting solution contains a kind and amount of ions which are correlated as specified with the composition of coal being treated. As known to those skilled in the art, particularly suitable cations for use in such exchanges comprise hydrogen, calcium, and magnesium ions. Particularly suitable anions for such use comprise sulfate and, whenever the chlorine concentration in non-water soluble components of the coal is suitably low, chloride ions. Nitrogen-containing substances such as ammonium ions or nitrate or other nitrogen-containing anions are typical of substances capable of forming atmospheric pollutants during oxidation of the coal and should be avoided.

In general, the aqueous solution of either a strong or weak electrolyte suitable for use in the present invention can be formed by mixing with an aqueous liquid (such as the liquid with which the coal is to be contacted, or the liquid with which the coal is wetted following a water-wash, or the liquid with which the coal

is slurried) substantially any water-miscible fluid which comprises or contains at least one compound capable of forming an aqueous solution of electrolyte. Examples of such compounds include gaseous, liquid or dissolved or

solid, acid anhydrides of strong or weak acids, such as CO<sub>2</sub>, the anhydrides of acetic, or propanoic, or the like acids, SO<sub>2</sub>, SO<sub>3</sub>, H<sub>2</sub>SO<sub>4</sub>, HCl, dissolved and/or slurried calcium chloride, magnesium chloride, sulfurous or the like electrolyte precursors which are compatible with the other components of the aqueous electrolyte solution being formed. Liquid or gaseous CO<sub>2</sub> is particularly suitable as such an electrolyte-forming fluid to be injected into a pipeline containing an aqueous slurry of coal. Mixtures of electrolytes can also be used, if found in a convenient form, and if they can be administered at proper concentration levels.

In general, when conducting the present process as a two-stage operation, with one portion conducted in a convenient location prior to conducting a further treatment within a pipeline, it is desirable to conduct the first

portion with a strong electrolyte and the latter portion with a weak electrolyte. Where the chloride content of the coal is low enough it may be desirable to utilize a strong, but relatively noncorrosive, electrolyte such as calcium chloride in the pipeline treatment. In the pipeline treatment, it is advantageous to conduct the fluid which is (or contains) an acidic electrolyte precursor, through a separate conduit leading into and discharging within a central portion of a stream of coal slurry which is flowing within the pipeline. In addition, it is desirable to correlate the kind and concentration of the electrolyte precursor with the composition of the coal so that the pH of the resultant aqueous electrolyte solution will become high enough to substantially reduce the corrosivity of an acidic solution by the time that solution has diffused into contact with the walls of the pipeline.

An ion exchanging of coal in an aqueous electrolyte solution generally leaves the coal wetted with an aqueous solution of salts which tend to become deposited on or otherwise attached to the coal as the water evaporates, unless the ion-exchanged coal receives an additional washing with substantially deionized water. Where the coal contains a relatively low concentration such as less than about 0.3%w of chlorine (as ions and/or atoms of non-water-soluble components) an aqueous electrolyte comprising calcium chloride or mixtures of it with acids which form water-soluble calcium salts are particularly suitable electrolyte solutions, particularly for uses in situations where the pH of the coal ion exchanging solution must be kept relatively non-acidic. Since most coals contain less than 0.3%w chlorine, it follows that CaCl<sub>2</sub> and its mixtures can be useful exchanging agents in numerous applications.

In a preferred procedure coal ground to particles of less than about  $\frac{3}{4}$ " diameter is water-washed by a process involving immersing the coal in an aqueous liquid which is substantially free of sodium ions. The washed coal is mechanically separated from the liquid in at least two fractions. Fraction (A) comprises relatively large coal particles capable of being settled by gravity from the liquid in a feasibly short time. Fraction (B) comprises the particles which are too fine for such a desirably rapid mechanical separation. The particles of fraction (A) are separately ion-exchanged with an aqueous electrolyte, then mixed with an aqueous slurry of the particles of fraction (B). The resulting mixture is preferably subjected to an additional ion-exchange.

What is claimed is:

1. In a process for reducing the sodium concentration of coal by contacting the coal with an aqueous solution of strong electrolyte, an improvement comprising:
  - initially washing the coal with water which is substantially free of sodium ions, to remove water-soluble materials which contain sodium ions;
  - ion-exchanging the water-washed coal with an aqueous solution of strong electrolyte in which both the kinds and amounts of ions are correlated with the kinds and amounts of ion-exchangeable ions on the coal, so that said solution (a) is relatively free of sodium ions, (b) is sufficiently free of substances capable of forming atmospheric pollutants during an oxidation of coal so that the resultant total amount of those substances in the ion-exchanged coal is insufficient to cause significant pollution and (c) contains an amount of cations capable of exchanging with ion-exchangeable cations on the coal which amount is less than the stoichiometric amount of ion-exchangeable cations on the coal but is an amount which causes sodium ions to be selectively removed during the ion exchanging of the coal; and
  - conducting at least a significant proportion of said water-washing and/or ion-exchanging by flowing within a pipeline both a slurry of coal in aqueous liquid which is substantially free of sodium ions and a stream of fluid which comprises or contains at least one compound capable of forming an aqueous solution of electrolyte having the properties designated (a), (b) and (c) when mixed with the aqueous phase of said coal slurry.
2. The process of claim 1 in which particles of the water-washed coal are separated into fraction (A) comprising relatively large particles susceptible to desirably rapid mechanical separation from aqueous liquid and fraction (B) comprising a pumpable slurry of fine particles in aqueous liquid.
3. The process of claim 1 in which an initial portion of the ion-exchange treatment is conducted by contacting the water-wet coal with an aqueous solution of strong

electrolyte before conducting the ion exchange treatment within the pipeline.

4. The process of claim 1 in which said compound capable of forming an aqueous electrolyte in the fluid flowing within the pipeline forms a weak electrolyte.
5. The process of claim 4 in which the compound capable of forming an aqueous electrolyte in the fluid flowing within the pipeline is at least one member of the group consisting of  $\text{CO}_2$ ,  $\text{CaCl}_2$ ,  $\text{MgCl}_2$ ,  $\text{H}_2\text{SO}_3$ ,  $\text{H}_2\text{SO}_4$ ,  $\text{SO}_2$  or  $\text{SO}_3$ .
6. The process of claim 1 in which particles of the water-washed coal are separated into fraction (A) comprising relatively large particles susceptible to desirably rapid mechanical separation from aqueous liquid and fraction (B) comprising a pumpable slurry of fine particles in aqueous liquid;
- particles of fraction (A) are ion-exchanged by contacting them with the aqueous solution of strong electrolyte, slurred with aqueous liquid and flowed into a pipeline; and
- the slurry comprising fraction (B) and a stream of at least one compound capable of forming a weak or strong electrolyte in an aqueous solution are flowed into said pipeline and into contact with the ion-exchanged particles of fraction (A).
7. The process of claim 6 in which fraction (A) of coal is contacted with aqueous electrolyte solution at a weight ratio of 1 coal/3 solution to 1 coal/10 solution.
8. The process of claim 7 in which said weight ratio is 1 coal/4 solution to 1 coal/7 solution, and the combined fractions (A) and (B) are contacted in a pipeline for simultaneous transport and sodium removal at a weight ratio of 1 weight of coal per 1.3 weights of aqueous solution to 1 weight of coal per 4 weights of aqueous solution.
9. The process of claim 8 in which said ratios of weight of aqueous solution to weight of coal range from 1 to 1.5 to about 1 to 2.5.
10. The process of claim 1 in which the fluid comprising or containing said compound capable of forming an electrolyte comprises a gaseous fluid and portions of it are injected at a plurality of points along the pipeline.

\* \* \* \* \*